

Aug. 10, 1937.

J. A. BRANEGAN

2,089,182

PILE FABRIC CONSTRUCTION

Filed May 29, 1935



INVENTOR.  
JAMES A. BRANEGAN

BY

*Richards & Geier*  
ATTORNEYS

## UNITED STATES PATENT OFFICE

2,089,182

## PILE FABRIC CONSTRUCTION

James A. Branegan, Philadelphia, Pa.

Application May 29, 1935, Serial No. 23,988

4 Claims. (Cl. 28—1)

The present invention relates to an improved pile fabric and it particularly relates to a composite pile fabric the pile of which is wholly or largely composed of synthetic yarns, particularly 5 of cellulosic character.

The invention of the present application will be particularly described in connection with its application to a type of velvet known as transparent velvet.

10 An object of the present invention is to provide an improved pile fabric particularly of transparent velvet type which will be provided with a more durable and substantially resistant pile, which will be of enhanced durability and substantially improved wearing qualities and which may be made up to form dresses and other wearing apparel of superior appearance and quality.

Other objects will be obvious or will appear during the course of the following specification.

20 Although not limited thereto, the present invention is particularly applicable to pile fabrics of the type in which the pile is substantially completely composed of rayon, while the ground is composed partly of rayon and partly of natural silk, or wholly of rayon.

It has been found that the quality of pile fabrics having rayon piles may be particularly greatly improved by subjecting such piles to successive dyeing, oiling and plastic coating operations, the 30 coating operation being carried out with a plastic material which may be readily applied in a liquid, aqueous or organic solvent bath and which may be substantially hardened so as to be resistant to washing.

35 To give an example of the manner of preparing fabrics for these successive treatments, it has been found suitable to weave together a ground warp of a 60 to 70 turn natural silk in gum yarn and a filling of a rayon yarn having 40 to 45 turns 40 per inch, although a natural silk filling may also be employed.

The pile, however, is most satisfactorily formed of a relatively heavy multi-filament rayon yarn, preferably a yarn having more than 20 filaments 45 and a denier of more than 100. The number of filaments may conveniently range from 50 to 60 while the denier may range from 100 to 180 or more. A preferred pile material is a rayon yarn having about 40 filaments and over 140 denier and 50 having a twist of about 3 to 7 turns per inch.

In a preferred form of the present invention, a rayon pile, transparent velvet, after dyeing is subjected to a surfacing with a solution containing a water soluble synthetic resin of the type 55 known as the urea formaldehyde resins. This

resin is applied after the fabric has been passed through a water bath containing sulphonated olive oil, or the sulphonated olive oil may be added to the resin bath.

The resin solution is applied without nipping or mangling so it will lie upon the surface of the rayon pile ends and after vacuum extraction, the fabric is heated, preferably incidental to finishing, sufficiently to convert the resin into insoluble form. The fabric so treated not only is of enhanced quality but also is crush-proof, crease-proof and appears to be substantially waterproof.

Upon the accompanying drawing is shown typical transparent velvet construction with a pile warp 12, a ground warp 11 and a ground filling 15 10. After cutting the pile fibers are indicated at 13.

After the pile fabric has been woven it may be satisfactorily degummed by treatment in a hot or boiling alkaline soap solution and the fabrics 20 may then be satisfactorily dyed, the dyeing being carried out together with or subsequently to the degumming operation.

Then the fabric is subjected to an oiling operation which consists in passing the fabric through a bath of emulsified oil, which may include a sulphonated or sulphonated oily material, such as olive oil, menhaden oil, palm oil, mustard seed oil, pea seed oil, cocoanut oil, cottonseed oil, rape seed oil, castor oil, neat's-foot oil, peanut oil, lard oil, 25 tallow oil, elaine oil, corn oil, sperm oil, fish oil, and/or cod oil or mixtures thereof. The emulsion preferably should be of such a character so that the oil particles will be larger than the pores in the pile fibers whereby assurance is had that a 30 layer of oil will be deposited on the various fibers 35 of the pile without penetration into the fibers of the pile itself.

The oil should be of such a character as to emulsify readily in water, but it should not be 40 of such a character as to go into true solution or to form a dispersion of too fine particles.

The pile fabric which has thus been oiled and substantially completely coated with this oily material is then run through liquid aqueous or 45 other liquid, organic or solvent bath containing the plastic material in dispersion, suspension or solution.

Among the solution and suspensions which 50 may be employed are those having either a water base or an organic solvent base, and in suspension, solution or dispersion in said bases, there may be employed various types of plastic materials such as aluminum salts of high molecular weight, carboxy or sulfoaliphatic and/or aro- 55

matic compounds, gelatin, albumen, synthetic resins, natural resins, gums, rubber or latex, cellulose compounds, waxes, fats, starch, casein, sugar, camphor, phenols, cresols and so forth.

5 Among the baths which may be satisfactorily employed are aqueous solutions of gelatin, glue and/or casein which may contain coagulating agents, such as dichromate or paraform. The coagulating agent, however, may be omitted in 10 the bath and the gelatin coated pile then subsequently subjected to treatment with a coagulating bath or atmosphere.

There also may be employed aqueous solutions of urea, thio-urea and formaldehyde compounds, 15 or phenol, cresol or other formaldehyde compounds, preferably in water soluble condition.

If desired the resins or other plastic materials may be placed in suspension or emulsion in the oil treating bath so that the oil and resin or 20 other plastic material will be deposited together on the outside of the fibers in the manner above described.

Among the aqueous solutions which may be utilized are solutions of methylol urea, and di- 25 methylol urea, preferably in 14 to 25% concentration, said solutions preferably being maintained at a pH of between 6 and 7, or between 5 and 7.

The fabric after removal from the plastic coating bath is then subjected to a process of vacuum extraction with the pile preferably extending toward the source of the vacuum. It is most important that during this process of impregnation and subsequent thereto not to subject the fabric 35 to any mechanical treatment or operation which might cause the resin or the oil to penetrate within the fibers or within the various strands making up the fabric, as otherwise an unsatisfactory treatment will be obtained. A wringer operation is used to remove the excess solution in some instances, to lessen the load on the vacuum extractor.

It is usually desirable, however, to omit all squeezing or wringing out operations.

45 The fabric after thus being impregnated and extracted is provided with an all-encompassing surfacing of oil in which is carried the plastic or other resinous material.

The pile fabric is then subjected to a drying operation. During this drying operation a temperature between 150 and 250° F. may be employed but preferably the temperature of 200° F. is not exceeded. The fabric is preferably subjected to this drying temperature for about 5 55 minutes, while the pile is being brushed in different directions and then afterwards the fabric again is subjected to the same temperature for a similar length of time without brushing the pile. The first heating operation should be sufficient to dry the fabric, while the second operation should be sufficient to harden and render insoluble the pile surfacing film.

The final fabric will be of satisfactory high 65 quality and may be most readily made up into dress fabrics. The pile will be somewhat stiffened without detracting from the quality of the fabric and at the same time it will be most durable and resilient and will stand up over long periods of time.

70 It also is possible to treat yarns and/or fabrics of silk, cotton, rayon, wool, worsted or other materials according to the present application, and also possible to treat other than pile fabrics by the process of the present application to obtain 75 a yarn or fabric of improved character, and en-

hanced appearance, both in regard to the wear and feel, flexibility and durability, and of improved drape.

It is also possible to treat fabrics, in some instances, after they have been treated according to the process of the present application in various manners, such as to color them, waterproof them, to fireproof them and so forth, which other finishing operations may also, if desired, be combined with the treating operations of the present 10 application.

It is also possible to treat the ground pile warp and also if desired the ground warp and ground filling with one of the plastic materials above before weaving, as a size, in which case if desired 15 the after treatment with the resin may be eliminated or the treatment of the fabric in a resin bath may be decreased so as to give a lesser coating of the fabric.

Where a waterproofing treatment is combined 20 with the principal treatment of the present application, such waterproofing effect may be attained by combining with the plastic material a high molecular weight aliphatic waxy, oily or fatty material, which may be put into the treating bath in the form of an emulsion if desired.

This high molecular weight material may also be utilized in the form of its sulphonic or carboxylic acid and caused to precipitate upon the fibers in the form of its aluminum or other heavy 25 metal salts.

It is also possible to enhance the properties of the fabric according to the present invention by treating the fabric with parchmentizing or mercerizing agents, which might tend to form a converted cellulosic material on the rayon fibers and this treatment may be carried out on the rayon yarn before it is woven into the final fabric. For example, treatments with carbon bisulphide and caustic alkali with combinations of acetic 40 acid and acetic anhydride, with caustic alkali and with etherifying and esterifying agents may well enhance the quality of the fabric. A similar surface effect upon the fabric may be obtained by directly treating the fabric with cellulosic compounds such as cellulose acetate, cellulose nitrate or cellulose xanthate.

It is to be understood that many alternative and modified processes and fabrics may be produced according to the disclosure of the present application and it is intended to include all such alternatives and modifications as may come within the scope of the appended claims.

What is claimed is:

1. A process of treating transparent velvet fabrics having a rayon pile to improve their quality and make them crush proof, which comprises providing the woven fabric in the form of gray goods, treating the gray goods to remove the coatings and gum therefrom, dyeing the fabric, and then treating the fabric so as to deposit upon the rayon pile ends a coating containing an emulsified sulphonated fatty oil and a water soluble synthetic resinous material, the oil being deposited from aqueous emulsion and the resinous material being deposited from a solution in an aqueous medium through which the fabric is passed, extracting the excess aqueous liquid, drying the fabric, finishing the fabric by brushing the pile so that it will take a desired conformation and then heating the fabric sufficiently to convert the water soluble synthetic resinous material into water insoluble condition.

2. The process of claim 1 in which the gray goods are composed of a ground warp of 60 to 70 75

turns natural silk in gum, in which the pile warp is composed of a multi-filament rayon yarn, and in which the filling is composed of a rayon yarn having a relatively high twist, in which the urea formaldehyde resin is employed in 14 to 25% concentration in the bath having a pH of between 5 and 7, in which the oily material is a sulphonated olive oil and in which during the insolubilizing of the resin, the fabric is subjected to a temperature of between 150° to 250° F. for a few minutes.

3. An improved crush proof transparent velvet textile fabric provided with a rayon pile in which

the rayon pile ends are coated with a composition consisting of a sulphonated fatty oil and heat-insolubilized, water-soluble synthetic resinous composition, said fabric retaining substantially its original suppleness.

4. An improved crush proof rayon pile transparent velvet fabric having substantially its original suppleness, the rayon pile ends being coated with an emulsifiable sulphonated olive oil and a water soluble synthetic urea formaldehyde resin, the latter being insolubilized by the baking.

JAMES A. BRANEGAN.